

## UNITED STATES PATENT OFFICE

WILLIAM C. SCHROEDER, OF HARRISBURG, PENNSYLVANIA, ASSIGNOR TO INDELIBLE COLORATION CORPORATION, OF NEW YORK, N. Y., A CORPORATION OF NEW YORK

## STAINING INK

No Drawing. Application filed March 29, 1922, Serial No. 547,820. Renewed February 4, 1929.

This invention relates to the art of printing on hard fusible materials, such as vitrics, ceramics, and metallic materials, and my improvements consist, first, in the production of an ink which is capable, by fusion, of becoming permanently associated, in the manner of a stain, with the surface of the material upon which it is imposed; and, secondly, in the application of the said fusible ink to the surface intended for its imposition by the act of printing it thereon direct, and then in subjecting the printed material to a temperature sufficiently high to fuse the ink imposed thereon and render the surface of the material capable of absorbing the fused ink to the extent that the ink penetrates the material, thereby representing the printed impression thereon in ineradicable fashion, and without presenting any excrescence from the surface.

In carrying out my invention I provide a fusible ink which is composed of a suitable vehicle that is impregnated with various metallic oxides, such for example as manganese, cobalt, uranium, etc., to furnish the desired color.

The base of the vehicle employed by me may be linseed oil, which is to be boiled and to have the scum removed therefrom while boiling. During the boiling operation certain other ingredients are to be added, namely, red lead, balsam of sulphur, Barbados tar, capivi balsam, oil of amber, acetate of lead and rosin.

This composition has been found by me in practice to constitute a satisfactory vehicle for the metallic oxides in the production of my fusible printing ink, and I have also found in practice that the vehicle may include the said ingredients in substantially the following proportions.

|                      | Ounce |
|----------------------|-------|
| Linseed oil          | 16    |
| Red lead             | 2     |
| 45 Balsam of sulphur | 4     |
| Capivi balsam        | 1/2   |
| Barbados tar         | 4     |
| Oil of amber         | 1/2   |
| Acetate of lead      | 1/2   |
| 50 Rosin             | 1/2   |

In preparing the said vehicle I have found it desirable to boil the linseed oil for about two hours, carefully removing the scum that may be thrown up, adding red lead, and burning off all greasy particles. The other named ingredients are also added to the linseed oil while boiling.

Following the boiling the vehicle is allowed to simmer, and while simmering the metallic oxide is added to provide the desired coloring matter, thereby completing the preparation of the ink, which may then be allowed to cool, and ground in a printing ink mill, when it will be found to have a consistency suitable for printing ink.

The ink thus prepared may then be applied to the surfaces of such substances as vitrics, ceramics, metals, metallic alloys and other hard fusible materials, the method of application being such as is generally known in the printing arts; although it will be appreciated that, since the printing is to be performed on hard surfaces, the impressing medium by which the ink is to be transmitted to such surfaces is preferably of relatively soft material.

In this act of printing, the inked impression is deposited upon the hard surface in the same manner as types or other printing media would impose impressions, with ordinary printing ink, upon paper.

The hard fusible material, thus printed, is then subjected to heat at a sufficiently high temperature to fuse the ink, which also serves to heat the hard, fusible material, bearing the printed impression, to a point at which it permits surface absorption of the fused ink, somewhat in the same manner as a stain is absorbed by wood.

The temperature at which I have successfully fused my improved ink to amalgamate it with the surface of hard, fusible material has been about 450° F. All the organic ingredients of the ink will have been completely consumed before this temperature is reached, leaving only the unvolatilized metallic elements, including the pigments employed, as representative of the prepared ink in the finished product.

While I have referred to my improved im-

65

60

65

70

80

85

90

95

100

- pression creating material as an ink, being warranted in so styling it on account of its facility of application being comparable to that of ordinary printer's ink, I am equally entitled to refer to this product as a stain, because, under fusion, it adapts itself to surface absorption by hard fusible materials somewhat as ordinary stain does with wood. Therefore I believe it appropriate to identify my improved ink product as a fusible staining-ink, and also to identify the new art which has come into being through the new material, as the art of stain-printing on hard fusible materials.
15. Variations within the spirit and scope of my invention are equally comprehended by the foregoing disclosure.

I claim:—

20. A fusible staining-ink composed of mineral oxides having as a vehicle linseed oil with which are compounded, red lead, balsam of sulphur, Barbados tar, capivi balsam, oil of amber, acetate of lead and rosin.

25. Signed at the borough of Manhattan, in the city, county and State of New York, this 27th day of March, 1922.

WILLIAM C. SCHROEDER.

30

35

40

5

10

15

20

25

30

35

40

45

50

55

60

65